

# UNITED STATES PATENT OFFICE.

ALBERT H. KING AND BERT CONNERS, OF TOLEDO, OHIO.

## DAMP-PROOF PAINT.

1,277,425.

Specification of Letters Patent.

Patented Sept. 3, 1913.

No Drawing.

Application filed October 17, 1917. Serial No. 197,612.

To all whom it may concern:

Be it known that we, ALBERT H. KING and BERT CONNERS, citizens of the United States, and residents of Toledo, in the county of Lucas and State of Ohio, have invented a certain new and useful Damp-Proof Paint; and we do hereby declare the following to be a full, clear, and exact description of the invention, such as will enable others skilled in the art to which it appertains to make and use the same.

This invention relates to a paint, and has for its object the provision of a damp-proof paint, which is particularly intended for use on damp surfaces, such, for instance, as freshly plastered walls, and which will dry quickly and while the surface which it covers is still damp, without cracking, peeling or chipping off.

20 The paint in its preferred embodiment comprises—

|                                  |     |
|----------------------------------|-----|
| White lead                       | 40% |
| Ped plaster                      | 20% |
| 25 Plaster of Paris              | 10% |
| Chinawood oil                    | 9%  |
| Coach varnish (preferably No. 1) | 3%  |
| Turpentine                       | 3%  |
| Naphtha                          | 15% |

30 These ingredients, with the exception of the naphtha, after being thoroughly mixed together, are thinned by the introduction of the naphtha.

The white lead, ped plaster and plaster of Paris form the base or body of the paint. If desired, silica and whiting may be substituted together for the plaster of Paris and should therefore be considered as an equivalent of plaster of Paris so far as the present invention is concerned. Ped plaster, which is the commercial name for a cement or plaster-like substance, contains a mixture of substantially 66% plaster of Paris and 33% lime. It is thus apparent that the paint

mixture contains approximately 7% lime and 23% plaster of Paris.

The paint embodying our invention will dry very quickly on either dry or damp surfaces, and is particularly intended for use as a first coat for damp surfaces, and may be applied to damp plastered walls shortly after plastering or the application of the putty coat thereto, and will quickly dry and form a hard dry surface over the plaster or putty coat and firmly adhere thereto irrespective of the condition of the plaster. This paint is also particularly adapted for use on the hulls of boats and on other surfaces which it is desired to render waterproof or to have moisture excluded therefrom.

If desired, a coloring ingredient may be added to the compound to give it the desired color.

It is to be understood that while we have particularly described the ingredients and proportions thereof embodied in a preferred form of the invention, the invention is not restricted thereto, but is entitled to numerous modifications without departing from the spirit of the claims.

Having thus described our invention, what we claim as new, and desire to secure by Letters Patent, is—

1. A damp-proof paint, comprising white lead, lime, plaster of Paris, Chinawood oil, varnish, turpentine and naphtha, substantially as described.

2. A damp-proof paint, comprising white lead, lime, plaster of Paris, and oil ingredient, varnish and turpentine mixed together in substantially the proportions designated and thinned with naphtha.

In testimony whereof we have hereunto signed our names to this specification.

ALBERT H. KING.  
BERT CONNERS.

Copies of this patent may be obtained for five cents each, by addressing the "Commissioner of Patents, Washington, D. C."

It is hereby certified that in Letters Patent No. 1,277,425, granted September 3, 1918 upon the application of Albert H. King and Bert Connors, of Toledo, Ohio, for an improvement in "Damp-Proof Paint," an error appears in the printed specification requiring correction as follows: Line 80, claim 2, for the word "and" read *an*; and that the said Letters Patent should be read with this correction therein that the same may conform to the record of the case in the Patent Office.

Signed and sealed this 8th day of October, A. D., 1918.

[SEAL.]

R. F. WHITEHEAD,

*Acting Commissioner of Patents.*

Cl. 134—39.